

Patented July 20, 1926.

1,592,961

# UNITED STATES PATENT OFFICE.

HEINRICH RÖSSNER AND ERNST RUNNE, OF HOCHST-ON-THE-MAIN, GERMANY, AS  
SIGNORS TO GRASSELLI DYESTUFF CORPORATION, OF NEW YORK, N. Y., A COR-  
PORATION.

## BASIC CHROMIC SALTS AND PROCESS OF MAKING SAME.

No Drawing. Application filed December 16, 1925, Serial No. 75,857, and in Germany November 8, 1924.

Solutions and suspensions of basic chromic salts—that is to say of those salts which contain at the most 140 parts of sulfuric anhydride ( $\text{SO}_3$ ) to 152 parts of chromic oxide ( $\text{Cr}_2\text{O}_3$ ) if the acid combined with the chromium is calculated as  $\text{SO}_3$ —when dried in the usual manner for instance by means of a roller-apparatus yield products which can be dissolved in water only with difficulty. Apart from any additions, foreign salts etc., the solubility of the basic chromic salts is the lower with one and the same acid the more basic the salts are and the higher the temperature is at which they are dried. For instance a solution of basic chromic sulfate which contains 120 parts of  $\text{SO}_3$  to 152 parts of  $\text{Cr}_2\text{O}_3$  and has been dried in the usual manner, gives a product containing about 37 per cent of  $\text{Cr}_2\text{O}_3$  which is almost insoluble in cold water and dissolves only gradually when covered over with hot water. The said chromic salt can be dissolved only after having been soaked for a prolonged time in cold water and subsequently heated.

Now we have found that chromic salts of the above indicated high basicity can be obtained in a dry state and in a form in which they are readily soluble even in cold water and most easily soluble in hot water, by exposing the solutions or suspensions of the chromic salts in a finely subdivided, particularly in an atomized state, to a hot current of gas or, preferably, of air. For instance a sulfate of the last mentioned composition which has been dried in the manner just described at 60–70° C. dissolves comparatively more readily than a product which has been dried by means of a roller apparatus. The said chromic salt dried on a roller apparatus dissolves in cold water only to a very small extent and in hot water to the extent of 10–20 per cent, during the time that the preparation dried by our new process, which is at once soluble in hot water, is completely dissolved.

This excellent solubility of chromic salts of such a high basicity and containing such a high percentage of chromic oxide as above indicated has not been known hitherto and offers a great advantage to the tanner. He is not compelled to prepare his chromium solution a long time before he proceeds to the tanning operation by soaking the prod-

uct for a prolonged time and subsequently heating as above mentioned, but he can prepare this solution immediately before he begins with the tanning operation. Furthermore, he can easily dissolve the basic chromic salt in the course of the tanning operation if, for some reason or other, he wishes to add a further quantity of the chromic salt to the tanning liquor.

By our new process the chromic salts are obtained in such a loose and finely subdivided state that they do not require any further grinding before they are used. They are also entirely free from injurious admixtures of metals, such as iron, which when a roller apparatus is used for the drying operation are always dissolved to some extent.

The solutions of the basic chromic salts may be prepared by dissolving chromic hydroxide or basic chromic hydroxides in acids or by reducing chromates or by any other known method. Their composition may greatly vary. There may be used salts of a single acid or of a mixture of several acids. There may also be employed inorganic or organic acids, such as formic acid, acetic acid or the like. The chromic salt solutions to be evaporated according to our new process may also contain other substances such, for instance, as a salt, sodium sulfate or the like, without impairing the result. During the drying process the temperature may vary within wide limits.

The following example serves to illustrate our invention:

50 kg. of chromic oxide, which may for instance be in the form of a precipitate of chromic hydroxide, are dissolved by means of 60,2 kg. of sulfuric acid of 60° Bé. and 21,8 kg. of hydrochloric acid of 20° Bé, atomized in any suitable manner and dried by means of a current of hot gasses or air of, for instance, 60–70° C. In this manner a green powder containing about 36 per cent of  $\text{Cr}_2\text{O}_3$  is obtained which dissolves in a very short time in cold water and immediately in hot water.

In the foregoing description and in the following claims we understand by the term "solutions of a basic chromic salt" to be dried also such solutions in which the chromic salt is only partly dissolved or is suspended therein.

We claim:—

1. The process of preparing readily soluble basic chromic salts, which consists in treating solutions of chromic salts, which contain not more than so much of an acid to 152 parts by weight of  $\text{Cr}_2\text{O}_3$ , as is equivalent to 140 parts by weight of  $\text{SO}_3$ , in a finely subdivided condition with a hot gas stream. 25
- 10 2. The process of preparing readily soluble basic chromic salts, which consists in treating a basic chromic salt, which contains so much of  $\text{SO}_3$  and of Cl to 152 parts of  $\text{Cr}_2\text{O}_3$ , that the total quantity is equivalent to not more than 140 parts by weight of  $\text{SO}_3$ , in a finely subdivided condition with a hot gas stream. 30
- 15 3. The process of preparing readily soluble basic chromic salts, which consists in treating solutions of chromic salts, which contain not more than so much of an acid to 152 parts by weight of  $\text{Cr}_2\text{O}_3$ , as is equivalent to 140 parts by weight of  $\text{SO}_3$ , in a finely subdivided condition with a hot gas stream. 35

to 152 parts of  $\text{Cr}_2\text{O}_3$ , that the acid is equivalent to 140 parts of  $\text{SO}_3$ , in a finely subdivided condition with a hot gas stream of a temperature of 60–70° C.

4. A dry basic chromic salt which contains not more than so much of an acid to 152 parts by weight of  $\text{Cr}_2\text{O}_3$ , as is equivalent to 140 parts of  $\text{SO}_3$ , and which are readily soluble in cold water and dissolve immediately in hot water.

5. A dry basic chromic sulfate-chloride which contains not more than so much of the acid radicals thereof to 152 parts of  $\text{Cr}_2\text{O}_3$ , as is equivalent to 140 parts of  $\text{SO}_3$ , which substance readily dissolves in cold water, and immediately in hot water. 35

In testimony whereof, we affix our signatures.

HEINRICH RÖSSNER.  
ERNST RUNNE.